



US006436883B1

(12) **United States Patent**  
Nich

(10) **Patent No.:** **US 6,436,883 B1**  
(45) **Date of Patent:** **Aug. 20, 2002**

(54) **HYDRAULIC AND GEAR LUBRICANTS**

(75) Inventor: **Edward Chung-Yit Nieh, Austin, TX (US)**

(73) Assignee: **Huntsman Petrochemical Corporation, Austin, TX (US)**

(\*) Notice: Subject to any disclaimer, the term of this patent is extended or adjusted under 35 U.S.C. 154(b) by 0 days.

(21) Appl. No.: **09/827,526**

(22) Filed: **Apr. 6, 2001**

(51) Int. Cl.<sup>7</sup> ..... **C10M 107/34**

(52) U.S. Cl. ..... **508/579; 508/539; 508/562**

(58) Field of Search ..... **508/579**

(56) **References Cited**

U.S. PATENT DOCUMENTS

|             |           |                         |            |
|-------------|-----------|-------------------------|------------|
| 2,403,067 A | 7/1946    | Fischer et al.          | 252/51     |
| 2,892,854 A | 6/1959    | Hommer                  | 260/404    |
| 2,967,831 A | 1/1961    | Hommer                  | 252/77     |
| 4,151,101 A | 4/1979    | Anzenberger, Sr. et al. | 252/49.6   |
| 4,208,293 A | 6/1980    | Zaweski                 | 252/51.5 A |
| 4,293,432 A | 10/1981   | Papay et al.            | 252/49.9   |
| 4,557,846 A | 12/1985   | Wisotsky                | 252/51.1 A |
| 4,828,737 A | * 5/1989  | Sandberg et al.         | 508/579    |
| 5,259,970 A | * 11/1993 | Kanamori et al.         | 252/73     |
| 5,415,896 A | * 5/1995  | Mulvihill et al.        | 427/388.4  |
| 5,543,068 A | * 8/1996  | Kaimai et al.           | 252/68     |

5,559,087 A \* 9/1996 Halsrud et al. .... 508/579  
5,711,896 A \* 1/1998 Kaimai ..... 252/68  
6,133,211 A \* 10/2000 Cobianco et al. .... 508/579  
6,255,263 B1 \* 7/2001 Ryan ..... 508/579

OTHER PUBLICATIONS

Union Carbide technical bulletin for UCON® Hydraulic Fluid WS-34 (1991).

“Field Experience with a new Generation polyether polyol hydraulic fluid” from American Chemical Technologies, Inc. (date unknown, but the date at the top of our fax is Mar. 1, 2000).

\* cited by examiner

Primary Examiner—Ellen M. McAvoy

(74) Attorney, Agent, or Firm—Russell R. Stolle; Ron D. Brown; Christopher J. Whewell

(57) **ABSTRACT**

Provided herein are functional fluid compositions useful in hydraulic fluid and gear oil formulations. The formulations according to the invention include a predominant amount of at least one polyoxyalkylene glycol derived from the addition polymerization of an alcohol in the presence of an alkylene oxide mixture which contains a substantial amount of ethylene oxide. Fluids according to the invention exhibit suitable lubricity and stability characteristics and are generally water soluble to a degree sufficient to preclude formation of a sheen on the surface of a body of water into which a fluid according to the invention is brought into contact.

**20 Claims, No Drawings**

1

## HYDRAULIC AND GEAR LUBRICANTS

## FIELD OF THE INVENTION

The present invention relates to hydraulic fluids useful in a wide variety of applications where a hydraulic fluid is employed to transmit fluid pressure. The invention relates more particularly to hydraulic fluids which are intended to be used in locations near environmental water sources, such as streams, rivers, lakes, and oceans. The fluids according to the invention possess strong dispersant qualities sufficient to leave no sheen in cases of their accidental release to environmental water sources. The hydraulic fluids of the invention are extremely low in toxicity to aquatic life and thus pose a minimal risk to ecosystems.

## BACKGROUND

Hydraulic fluids are used in systems which are generally well-known in the art for providing a means for transmitting any applying large forces to moveable mechanical components, while retaining a great degree of flexibility and control. Such systems are used in most forms of mechanized motion to transmit, transform and control mechanical work. They are part of a major technical discipline known to those skilled in the art as "fluid power technology".

A typical hydraulic system includes the following components: 1) a force-generating unit that converts mechanical energy into hydraulic energy, such as a pump; 2) a hydraulic fluid; 3) piping for transmitting fluid under pressure; 4) a unit that converts the hydraulic energy of the fluid into mechanical work, such as an actuator or fluid motor; 5) A control circuit with valves that regulate flow, pressure, direction of movement, and applied forces; and 6) a fluid reservoir that allows for filtration and/or separation of any particulate debris or water before returning the clean fluid to the system. Thus, the fluid is in contact with each mechanical component of the system used for transmitting mechanical energy, including metallic components which may come into direct physical contact with one another.

It is generally accepted that hydraulic fluids can be defined as any liquids which are necessary for the proper functioning of a hydraulic system. The primary function of the fluid is to transmit force which is applied at one point in the system to some other location in the system, and to quickly produce desired changes in the direction or the magnitude of that force. Hydraulic systems using such suitable fluids are very common and have numerous applications in industry and daily life, including uses in automotive systems such as brakes, clutches, and transmissions, in industrial equipment for applications such as pressing, molding, mining, metal forming and positioning, excavation equipment such as backhoes, in devices such as elevators, and in the transportation industry for many control and motive systems in ships and aircraft. The art of hydraulic fluid formulation contains several technical references which describe hydraulic fluids which are based upon hydrocarbon oils. Such systems include those described in U.S. Pat. Nos. 2,403,067; 2,892,854; 2,967,831; 4,151,101; 4,208,293; 4,293,432; and 4,557,846, the entire contents of each of which are herein incorporated by reference thereto.

For optimal functioning, a hydraulic fluid must be relatively incompressible and must flow readily. In addition, there are a number of secondary functions provided by hydraulic fluids, which functions are extremely important for successful system operation, including adequate lubricity for moving parts, stability under anticipated conditions of use, compatibility with materials used to construct the

2

hydraulic system, and the fluids should have the ability to protect system components against chemical reaction with materials which may enter the system.

Additives to the fluid which protect system components against chemical reaction are frequently called "corrosion inhibitors". Corrosion can result from the formation of reactive decomposition products of the fluid itself, from components of the fluid (e.g., additives) which are corrosive, or from the entry of contaminants into the hydraulic system.

10 In the case of hydraulic fluids which are based upon hydrocarbon oils, an environmental problem arises when such fluids come into contact with environmental water sources in that at least a portion of the oils tend to float on the surface of the water and create an unsightly sheen which may extend or be visible for great distances. This is known to be the case even when the total amount of the oil accidentally spilled is relatively small, and the concentration of the oil on surface of the water poses potential harm to 15 aquatic life forms. Such situations have in the past commonly arisen for ships at sea, when there is a leak of a hydraulic fluid used in one of the ship's operating systems, and in general in any situation where hydraulic fluids are used in close proximity to environmental water sources, such as oil drilling platforms, paper mills, and amusement parks. As the United States government has promulgated 20 rules concerning releases of materials that useful as hydraulic fluids in Title 40 of the Code of Federal Regulations, section 110, an increased level of awareness of issues surrounding spills of hazardous oils has become manifest in 25 recent years. In response with such rulemaking, many users of hydraulic oils have undertaken to employ special precautions in their handling and use of hydraulic fluids. Clearly, if formulations of hydraulic fluids were available that do not 30 form a sheen on the surface of water into which such fluids came into contact and which are environmentally benign, such fluids would be welcomed by all persons to whom such 35 fluid types are of practical use.

## SUMMARY OF THE INVENTION

The problems associated with the use of and release into environmental waters of water-immiscible, hydrocarbon oil based hydraulic oil formulations may be eliminated by the use of a liquid composition according to the present invention, which comprises water-soluble polyoxyalkylene glycols having either of the general formulae:



in which x is selected from any whole integer 1, 2, 3, 4, or 5; y is selected from 1 or 2; and m is an integer sufficient to provide a molecular weight in the range of between about 450 and 5000. Such materials are used in combination with a carboxylic acid having between about 6 and 18 carbon atoms per molecule of carboxylic acid, an amine, and optionally, an extreme pressure additive to provide a composition according to the invention. Since the physical properties and performance characteristics required of hydraulic fluids are similar to those required by gear oils in many applications, the formulations of the invention are of widespread applicability.

## DETAILED DESCRIPTION

The present invention comprises multi-component liquid compositions of matter which comprise a predominant

amount of a water-soluble polyoxyalkylene glycol having a pre-selected molecular weight of any value in the range of between 450 and 5000. When formulated according to the present invention, the functional fluids disclosed provide an excellent viscosity index which is greater than about 160. An especially preferred family of water soluble polyoxyalkylene glycol useful in the compositions of the present invention may also be one produced from alkoxylation of n-butanol with a mixture of alkylene oxides to form a random alkoxylated product which may be described by the either of the general formulae:



in which x may independently be any whole integer between 0 and 5, including 0 and 5; y may independently be any integer between 0 and 2, including 0 and 2; may independently be any whole integer between 1 and 5, including 1 and 5; p may independently be either 1 or 2; wherein m is an integer within the range suitable to provide a molecular weight of between 450 to 5000.

Functional fluids according to the invention possess a pour point of less than about -20° C., and exhibit compatibility with a wide range of anti-wear additive and extreme pressure additives. The formulations according to the invention also are devoid of fatigue failure that is normally expected by those of ordinary skill in the art when dealing with polar lubricant base stocks. This is evident from the comparison of the performance of similarly formulated butyl (polyoxypropylene only) based hydraulic fluids with those of the preferred form of the invention which are butyl (oxyethylene/oxypropylene).

It has been unexpectedly discovered that when normally highly oil soluble extreme pressure additives are used in a

concentration of 0.3 to 1.0% by mole of potassium hydroxide to the monomer(s) and at high temperature, as 100 degrees C. to 160 degrees C. It is well known fact that the potassium hydroxide being a catalyst is for the most part bonded to the chain-end of the produced polyalkylene oxide in a form of alkoxide in the polymer solution so obtained.

Useful as components in a formulation according to the present invention are those polyoxyalkylene glycols described by either of the general formulae:



in which x may independently be any whole integer between 1 and 5; and y may independently be either 1 or 2; and m is sufficient to provide a material having a molecular weight in the range of 450 to 5000.

An especially preferred family of water soluble polyoxyalkylene glycol useful in the compositions of the present invention may also be one produced from alkoxylation of n-butanol with a mixture of alkylene oxides to form a random alkoxylated product which may be described by the either of the general formulae:



formulation according to the invention and when a formulation according to the invention is spilled into a body of water, no sheen or oily layer on the surface of the water is visually detectable and the water surface is not discolored in any noticeable way. Such normally highly oil soluble extreme pressure additives include triisopropylphenyl phosphate.

#### The Polyoxalkylene Glycol Component

Polyoxalkylene glycols useful in the present invention may be produced by a well-known process for preparing polyalkylene oxide having hydroxyl end-groups by subjecting an alcohol or a glycol ether and one or more alkylene oxide monomers such as ethylene oxide or propylene oxide to addition polymerization while employing a strong base such as potassium hydroxide as a catalyst. In such process, the polymerization is commonly carried out under a catalytic

in which x may independently be any whole integer between 0 and 5, including 0 and 5; y may independently be either 1 or 2; z may independently be any whole integer between 1 and 5, including 1 and 5; p may independently be 1 or 2; and wherein m is an integer sufficient to provide a molecular weight in the range of 450 to 5000, subject to the provisos that at least one of x and z is equal to at least one and that at least one of y and p is equal to at least one.

It has been surprisingly found that hydraulic fluids prepared in accordance with the present invention which are made using a mixture of propylene oxide and ethylene oxide and n-butanol exhibit surprisingly low levels of toxicity while retaining adequate lubricity properties and dispersability characteristics for hydraulic fluid applications. Thus, preferred polyoxalkylene glycols useful in accordance with the present invention are those prepared using n-butanol as a starting material, and subjecting n-butanol to polymeriza-

tion conditions in the presence of a mixture of propylene oxide and ethylene oxide, in which the amount of propylene oxide in the gaseous mixture is preferably between 35.00% and 65.00% by weight based upon the total weight of the mixture, including every hundredth percentage therebetween, more preferably between 35.00% and 65.00% by weight based upon the total weight of the gaseous mixture, including every hundredth percentage therebetween, and most preferably between 45.00% and 55.00% by weight based upon the total weight of the gaseous mixture, including every hundredth percentage therebetween.

In order to produce a polyoxyalkylene glycol monobutyl ether with minimum polyoxyalkylene glycol contamination, it has been found beneficial to use an initiator for the polymerization, with a butanol-derived species that already contains one, two, or three alkylene oxide units per molecule such as a glycol ether represented by the formula:



wherein  $\text{R}_1$  is methyl or hydrogen and wherein  $m$  is independently selected from 1, 2, or 3 being especially preferred. These glycol ether initiators have a sufficiently low vapor pressure that allows the stripping of water from a mixture of the initiator and potassium hydroxide, and prevents unwanted polyoxyalkylene glycol by-product formation. Various suitable polyoxyalkylene glycols monobutyl ether for this invention are available from Huntsman Petrochemical Corporation having an office at 7114 North Lamar Blvd. in Austin, Tex. under the JEFFOX® tradename. Products of these alkoxylation reactions such as JEFFOX WL-170, JEFFOX® WL-260, JEFFOX® WL-660, and JEFFOX® WL-5000 having molecular weight ranges of about 450 to 5000 are useful as a component of formulations useful as a hydraulic fluid. JEFFOX® WL-170, has a number average molecular weight of about 450 and is useful as a component of formulations useful as a hydraulic fluid. JEFFOX® WL-260 has a number average of about 750 and is useful as a component of formulations useful as a hydraulic fluid. JEFFOX® WL-660 has a number average molecular of about 1800 and is useful as a component of formulations useful as a hydraulic fluid. JEFFOX(D WL-5000 has a number average of about 4200 and is useful as a component of formulations useful as a hydraulic fluid.

#### The Extreme Pressure Additive Component

For purposes of this specification and the appended claims the words "extreme pressure additive" means those particular chemical materials generally regarded by artisans of ordinary skill in the lubrication or tribology arts as being

useful as extreme pressure additives for ho lubricants, which include without limitation: sulfurized olefins, dithiophosphate salts of transition metals including without limitation such exemplary salts as zinc dithiophosphate and copper dithiophosphate, derivatives of alkylated phenols including mono or poly-alkyl phenol phosphates, organic phosphates, organic sulfur and chlorine compounds, sulfurized fats, other phosphates, sulfides, di-sulfides, and polysulfides. It is most preferred, however, that the extreme pressure additive comprise a trialkyl phenol phosphate such as those available under the tradename Durad 110, Durad 150, Durad 220, and Durad 300 from Great Lake Chemical Corp., of West Lafayette, Ind., USA; or those available under the trade name of IRGALUBE® from Ciba Specialty Chemicals of Basel, Switzerland. Durad 300 is an especially preferred trialkyl phenol phosphate.

#### The Amine Component

Compositions according to the invention also include an amine component, the function of which is to control corrosion by maintaining the overall pH of the lubricant in the alkaline range. Preferred amines for this use include primary amines, secondary amines, tertiary amines, cycloalkyl amines, aromatic amines, diamines, polyalkylene polyamines, and include all amines generally regarded by one of ordinary skill in the art as being useful for controlling corrosion of metal surfaces by either neutralizing acids produced during equipment operation or by acting as a metal deactivator. One especially preferred amine for use in compositions according to the invention is DIGLYCOLAMINE® Agent amine product because of its ability to impart both corrosion resistance and favorable toxicology profile. DIGLYCOLAMINE® Agent is available from Huntsman Petrochemical Corporation of Austin, Tex.

#### Toxicity to Aquatic Life

As mentioned, fluid compositions according to the invention exhibit an especially favorable low toxicity with respect to aquatic life, which is important from an environmental standpoint because leaks of functional fluids into the environment often occur at some point during either their storage, transportation, or use. Table I provides comparative data between monobutyl ethers which have been addition polymerized with different olefin oxides to different molecular weights. The olefin oxides used were propylene oxide ("PO") and ethylene oxide ("EO"). In one set of data, pure propylene oxide was used. In another set of data, a 50:50 mixture (molar basis) of propylene oxide and ethylene oxide was used in the polymerization. A third set of data was obtained for the butane di-ol based products in which a 75:25 molar mixture of EO to PO was employed during the polymerization.

TABLE I

| Type of Molecule | Oxide   | Molecular Weight | Poly-G ® Fluid Equivalents | Sturm Biodegradation | Concentrations (mg/L)                                              |                                                                   |                                                     |
|------------------|---------|------------------|----------------------------|----------------------|--------------------------------------------------------------------|-------------------------------------------------------------------|-----------------------------------------------------|
|                  |         |                  |                            |                      | 96-hr fathead minnow acute toxicity, LC <sub>50</sub> <sup>1</sup> | 48-hr Daphnia Magna acute toxicity, EC <sub>50</sub> <sup>2</sup> | Bacterial inhibition, IC <sub>50</sub> <sup>3</sup> |
| Monobutyl Ether  | 100% PO | 340              | WI-65                      | 84                   | 190                                                                | 450                                                               | 2,800                                               |
|                  |         | 740              | WI-165                     | 99                   | 86                                                                 | 250                                                               | 1,300                                               |
|                  |         | 1,020            | WI-285                     | 85                   | 37                                                                 | 69                                                                | 34,000                                              |
|                  |         | 1,550            | WI-625                     | 48                   | 20                                                                 | 26                                                                | 19,000                                              |
|                  |         | 2,490            | WI-1715                    | 23                   | 180                                                                | 520                                                               | >50,000                                             |

TABLE I-continued

| aquatic toxicity of various polyalkylene glycols |             |                  |                            |                      |                                                                    |                                                                   |                                                     |
|--------------------------------------------------|-------------|------------------|----------------------------|----------------------|--------------------------------------------------------------------|-------------------------------------------------------------------|-----------------------------------------------------|
| Type of Molecule                                 | Oxide       | Molecular Weight | Poly-G ® Fluid Equivalents | Sturm Biodegradation | Concentrations (mg/L)                                              |                                                                   |                                                     |
|                                                  |             |                  |                            |                      | 96-hr fathead minnow acute toxicity, LC <sub>50</sub> <sup>1</sup> | 48-hr Daphnia Magna acute toxicity, EC <sub>50</sub> <sup>2</sup> | Bacterial inhibition, IC <sub>50</sub> <sup>3</sup> |
| Monobutyl Ether                                  | 100% PO     | 520              | WS-100                     | 93                   | 3,200                                                              | 4,300                                                             | 18,500                                              |
|                                                  |             | 970              | WS-260                     | 65                   | 13,000                                                             | 5,400                                                             | 40,000                                              |
|                                                  |             | 1,700            | WS-660                     | 45                   | 24,500                                                             | 21,000                                                            | 32,000                                              |
|                                                  |             | 3,930            | WS-3520                    | 7                    | 11,900                                                             | 17,000                                                            | 10,000                                              |
| Di-ol                                            | 72:25 EO/PO | 2,470            | WT-1400                    | 71                   | 129,000                                                            | 88,000                                                            | 38,000                                              |
|                                                  |             | 12,000           | WT-90,000                  | 8                    | 65,000                                                             | 83,000                                                            | 94,000                                              |
| Water/glycol hydraulic fluid concentrate         | —           | —                | —                          | 57                   | 6,700                                                              | 1,400                                                             | 36,000                                              |
| Water/glycol hydraulic fluid                     | —           | —                | —                          | 64                   | 4,500                                                              | 4,800                                                             | 22,000                                              |

LC<sub>50</sub> = median lethal concentration (expected 50% mortality)EC<sub>50</sub> = median effect concentration (expected 50% loss of mobility)IC<sub>50</sub> = median inhibition concentration (expected 50% loss of respiration)

As is evident from the data in table I, polyoxyalkylene glycols produced using substantial amounts of ethylene oxide during the addition polymerization exhibit a much greatly reduced degree of toxicity with respect to those polyoxyalkylene glycols produced using only propylene oxide during the addition polymerization. Thus, the predominant ingredient in formulations according to this invention are seen to be of very low toxicity. Poly-G® is a trademark of Olin Corporation, and the various product equivalents indicate that these materials are available from Olin Corporation of Norwalk, Conn. The prefix WS, WI, and WT each mean water-soluble, water-insoluble, and water-thickening, respectively, and the number after the prefix indicates the approximate viscosity in Saybolt Universal Seconds (SUS) at 38° C. (100° F.).

## Fluid Formulations

30

-continued

35

40

55

60

|                       |     |
|-----------------------|-----|
| Decanoic acid         | 1.5 |
| DIGLYCOLAMINE ® Agent | 1.3 |
| Phenothiazine         | 0.5 |
| DURAD-300             | 1.5 |

## EXAMPLE 2

|                       |      |
|-----------------------|------|
| JEFFOX ® WL-170       | 20   |
| JEFFOX ® WL-260       | 75.2 |
| Decanoic acid         | 1.5  |
| DIGLYCOLAMINE ® Agent | 1.3  |
| Phenothiazine         | 0.5  |
| DURAD-300             | 1.5  |

## EXAMPLE 3

|                          |      |
|--------------------------|------|
| JEFFOX ® PPG-400         | 25   |
| JEFFOX ® WL-260          | 71.5 |
| N-phenyl-1-naphthylamine | 2.0  |
| DURAD-300                | 1.5  |

## EXAMPLE 4

|                       |      |
|-----------------------|------|
| JEFFOX ® WL-660       | 25   |
| JEFFOX ® WL-260       | 75.2 |
| Decanoic acid         | 1.5  |
| DIGLYCOLAMINE ® Agent | 1.3  |
| Phenothiazine         | 0.5  |
| DURAD-300             | 1.5  |

## EXAMPLE 1

JEFFOX ® PPG-400

25  
70.2

65

|                          |      |
|--------------------------|------|
| JEFFOX ® WL-660          | 20.5 |
| JEFFOX ® WL-260          | 77.5 |
| N-phenyl-1-naphthylamine | 2.0  |
| DURAD-300                | 1.5  |

|   |                       |      |
|---|-----------------------|------|
| 5 | Decanoic acid         | 1.0  |
|   | DIGLYCOLAMINE ® Agent | 0.85 |
|   | Phenothiazine         | 0.5  |
|   | DURAD-300             | 1.5  |

10

|                          |      |
|--------------------------|------|
| JEFFOX ® WL-660          | 33.5 |
| JEFFOX ® WL-260          | 63.0 |
| N-phenyl-1-naphthylamine | 2.0  |
| DURAD-300                | 1.5  |

|    |                  |      |
|----|------------------|------|
| 15 | EXAMPLE 12       |      |
|    | JEFFOX ® WL-660  | 23.0 |
|    | JEFFOX ® WL-5000 | 73.5 |
|    | Phenothiazine    | 2.0  |
|    | DURAD-300        | 1.5  |

20

|                  |       |
|------------------|-------|
| JEFFOX ® WL-660  | 77.15 |
| JEFFOX ® WL-5000 | 17.5  |
| Decanoic acid    | 0.85  |
| Phenothiazine    | 2.0   |
| DURAD-300        | 1.5   |

|    |                       |      |
|----|-----------------------|------|
| 25 | EXAMPLE 13            |      |
|    | UCON LB-165           | 39.0 |
|    | UCON LB-285           | 56.2 |
|    | Decanoic acid         | 1.5  |
|    | DIGLYCOLAMINE ® Agent | 1.3  |
|    | Phenothiazine         | 0.5  |
|    | DURAD-300             | 1.5  |

30

|                          |      |
|--------------------------|------|
| JEFFOX ® WL-660          | 79.0 |
| JEFFOX ® WL-5000         | 17.5 |
| Decanoic acid            | 0.85 |
| N-phenyl-1-naphthylamine | 2.0  |
| DURAD-300                | 1.5  |

35

|    |                       |      |
|----|-----------------------|------|
| 40 | EXAMPLE 14            |      |
|    | UCON LB-165           | 20.2 |
|    | UCON LB-285           | 75.0 |
|    | Decanoic acid         | 1.5  |
|    | DIGLYCOLAMINE ® Agent | 1.3  |
|    | Phenothiazine         | 0.5  |
|    | DURAD-300             | 1.5  |

45

|                       |       |
|-----------------------|-------|
| JEFFOX ® WL-660       | 42.65 |
| JEFFOX ® WL-5000      | 52    |
| Decanoic acid         | 1.0   |
| DIGLYCOLAMINE ® Agent | 0.85  |
| Phenothiazine         | 2.0   |
| DURAD-300             | 1.5   |

50

|    |                                                                                                                                                                                                                                                                                                                                    |
|----|------------------------------------------------------------------------------------------------------------------------------------------------------------------------------------------------------------------------------------------------------------------------------------------------------------------------------------|
| 55 | These formulations are useful as hydraulic fluids and gear lubes. The fluids of this invention are blends of the various components set forth. To produce a blended fluid in accordance with the invention, one merely mixes the various ingredients in a mixing kettle with gentle agitation until a homogeneous mixture results. |
|    |                                                                                                                                                                                                                                                                                                                                    |

|                  |      |
|------------------|------|
| JEFFOX ® WL-660  | 40.6 |
| JEFFOX ® WL-5000 | 55.9 |
| Phenothiazine    | 2.0  |
| DURAD-300        | 1.5  |

|    |                                                                                                                                                                                                                                                                                                                                                                                         |
|----|-----------------------------------------------------------------------------------------------------------------------------------------------------------------------------------------------------------------------------------------------------------------------------------------------------------------------------------------------------------------------------------------|
| 60 | One important property of formulations of hydraulic oils and gear lubes in general is that they should be relatively tolerant of impurities introduced thereinto, without suffering deleterious effects on their performance properties. In table II below are set forth results of the evaluation of the presence of various contaminants in a formulation according to the invention. |
|    |                                                                                                                                                                                                                                                                                                                                                                                         |

|                  |       |
|------------------|-------|
| JEFFOX ® WL-660  | 23.15 |
| JEFFOX ® WL-5000 | 73.0  |

TABLE II

effect of contaminants on various formulations according to the invention.

| Example # | Contaminant       | % contaminant | Drops in 2 Kg H <sub>2</sub> O | Observation     |
|-----------|-------------------|---------------|--------------------------------|-----------------|
| 2         | ECO-SAFE FR-46    | 3             | 5                              | no sheen        |
| 4         | ECO-SAFE FR-46    | 3             | 5                              | no sheen        |
| 6         | ECO-SAFE FR-46    | 3             | 5                              | no sheen        |
| 3         | ECO-SAFE FR-46    | 3             | 5                              | no sheen        |
| 13        | ECO-SAFE FR-46    | 3             | 1                              | two-phase       |
| 14        | ECO-SAFE FR-46    | 3             | 1                              | two-phase       |
| 2         | FM-HYDRAULIC AW46 | 3             | 5                              | no sheen        |
| 4         | FM-HYDRAULIC AW46 | 3             | 5                              | no sheen        |
| 6         | FM-HYDRAULIC AW46 | 3             | 5                              | no sheen        |
| 3         | FM-HYDRAULIC AW46 | 2             | 5                              | no sheen        |
| 13        | FM-HYDRAULIC AW46 | 3             | 1                              | two-phase       |
| 14        | FM-HYDRAULIC AW46 | 3             | 1                              | two-phase       |
| 2         | FM-HYDRAULIC AW68 | 2             | 5                              | no sheen        |
| 4         | FM-HYDRAULIC AW68 | 2             | 5                              | no sheen        |
| 6         | FM-HYDRAULIC AW68 | 2             | 5                              | no sheen        |
| 3         | FM-HYDRAULIC AW68 | 3             | 5                              | no sheen        |
| 13        | FM-HYDRAULIC AW68 | 3             | 1                              | two-phase       |
| 14        | FM-HYDRAULIC AW68 | 3             | 1                              | two-phase       |
| 3         | BIOHYDRAN         | 3             | 5                              | no sheen        |
| 4         | BIOHYDRAN         | 3             | 5                              | no sheen        |
| 6         | BIOHYDRAN         | 3             | 5                              | no sheen        |
| 3         | BIOHYDRAN         | 3             | 5                              | no sheen        |
| 13        | BIOHYDRAN         | 3             | 1                              | two-phase       |
| 14        | BIOHYDRAN         | 3             | 1                              | two-phase       |
| Reference | ECO-SAFE FR-46    | 100           | 1                              | dispersed sheen |
| Reference | FM-HYDRAULIC AW46 | 100           | 1                              | dispersed sheen |
| Reference | FM-HYDRAULIC AW68 | 100           | 1                              | dispersed sheen |
| Reference | BIOHYDRAN         | 100           | 1                              | floater         |
| 13        | None              | 100           | 1                              | two-phase       |
| 14        | None              | 100           | 1                              | two-phase       |

In Table II are listed the example number from the examples above which were evaluated for contaminant tolerance by observing the manifestation of a sheen, or lack thereof, on the surface of a 2 liter volume of water into which the denoted number of drops of a mixture comprising 97.0 grams of the particular formulation mixed with 3.0 grams of the contaminant are added. This information is valuable in selecting a given fluid formulation according to the invention as a replacement for a fluid of prior art, for it is often the case that it is not possible to completely evacuate a hydraulic system of its fluid when replacing the fluid, and in many cases residual amounts of used fluid remaining in the system can affect the performance of the replacement fluid. The contaminant listed as "ECO-SAFE FR-46" is a polyglycol product L available from American Chemical Technologies, Inc. of 46915 Liberty Drive, Wixom, Mich. 48393 and is generally employed as a hydraulic fluid. The contaminants listed as "FM-HYDRAULIC AW46" and "FM-HYDRAULIC AW46" are available from Citgo Petroleum Corporation of 1 Warren Place, Tulsa, Okla. and are mineral oil products which are generally employed as food-grade hydraulic fluids. The contaminant listed as "BIOHYDRAN" is Biohydron 46, available from Fina Lubricants of 400 Chism Place, Plano, Texas 75075 and is a vegetable oil that is generally employed as a bio-degradable, non-toxic hydraulic fluid.

The contaminants were tested alone in their neat forms to show that they are capable of producing a sheen on the surface of water into which they are added. In table II, the last two materials from examples 13 and 14 are those made using materials known as UCON LB-165 and UCON LB-285 in their formulations. These materials are available

from Union Carbide Corporation of Danbury, Conn., and are polyoxyalkylene glycols made from n-butanol and propylene oxide, i.e., no ethylene oxide is used during their manufacture. From these results it is seen that formulations made using these materials are not in the least bit compatible with water into which they may become mixed, as evidenced by the presence of two phases in the sheen test results.

In Table III are listed observations of the physical appearance of mixtures of various example formulations with the contaminants listed in the amount set forth on a weight basis.

TABLE III  
physical appearances of contaminated fluids according to the invention.

| Exam-<br>ple | #  | Contaminant       | Contaminant, % w/w |        |        |        |
|--------------|----|-------------------|--------------------|--------|--------|--------|
|              |    |                   | 2                  | 3      | 6      | 10     |
| 55           | 2  | ECO-SAFE FR-46    | clear              | clear  | clear  | clear  |
| 55           | 4  | ECO-SAFE FR-46    | clear              | clear  | clear  | clear  |
| 55           | 6  | ECO-SAFE FR-46    | clear              | clear  | clear  | clear  |
| 55           | 3  | ECO-SAFE FR-46    | clear              | clear  | clear  | clear  |
| 60           | 13 | ECO-SAFE FR-46    | clear              | clear  | clear  | clear  |
| 60           | 14 | ECO-SAFE FR-46    | clear              | clear  | clear  | clear  |
| 60           | 2  | FM-HYDRAULIC AW46 | clear              | cloudy | cloudy | cloudy |
| 60           | 4  | FM-HYDRAULIC AW46 | clear              | clear  | cloudy | cloudy |
| 60           | 6  | FM-HYDRAULIC AW46 | clear              | cloudy | cloudy | cloudy |
| 60           | 3  | FM-HYDRAULIC AW46 | clear              | clear  | cloudy | cloudy |
| 60           | 13 | FM-HYDRAULIC AW46 | clear              | clear  | clear  | cloudy |
| 60           | 14 | FM-HYDRAULIC AW46 | clear              | clear  | cloudy | cloudy |
| 60           | 2  | FM-HYDRAULIC AW68 | clear              | cloudy | cloudy | cloudy |
| 60           | 4  | FM-HYDRAULIC AW68 | clear              | clear  | cloudy | cloudy |
| 60           | 6  | FM-HYDRAULIC AW68 | clear              | cloudy | cloudy | cloudy |
| 60           | 3  | FM-HYDRAULIC AW68 | clear              | clear  | cloudy | cloudy |
| 60           | 13 | FM-HYDRAULIC AW68 | clear              | clear  | clear  | clear  |
| 60           | 14 | FM-HYDRAULIC AW68 | clear              | clear  | cloudy | cloudy |

TABLE III-continued

| Exam-<br>ple |             | Contaminant, % w/w |       |        |        |
|--------------|-------------|--------------------|-------|--------|--------|
| #            | Contaminant | 2                  | 3     | 6      | 10     |
| 3            | BIOHYDRAN   | clear              | clear | cloudy | cloudy |
| 4            | BIOHYDRAN   | clear              | clear | cloudy | cloudy |
| 6            | BIOHYDRAN   | clear              | clear | cloudy | cloudy |
| 3            | BIOHYDRAN   | clear              | clear | cloudy | cloudy |
| 13           | BIOHYDRAN   | clear              | clear | cloudy | cloudy |
| 14           | BIOHYDRAN   | clear              | clear | cloudy | cloudy |

Thus, the first line in table III sets forth the appearance of the composition according to formula 3 and having 2, 3, 6, and 10 percent by weight of the contaminant ECO-SAFE FR-46.

Evaluation of the performance of fluids provided by the invention for wear characteristics and extreme pressure properties were carried out in accordance with ASTM test methods D-2670 and D-3233. Each test run in duplicate, and results of the testing are tabulated in table IV:

TABLE IV

| Example No. | Wear Test (ASTM D-2670) | E. P. Test               |                               |
|-------------|-------------------------|--------------------------|-------------------------------|
|             |                         | Total Teeth Wear         | (ASTM D-3233)<br>Failure Load |
| 12          | run 1                   | 6                        | 1800                          |
|             | run 2                   | 8                        | 1750                          |
| 10          | run 1                   | 10                       | 1550                          |
|             | run 2                   | 10                       | 1700                          |
| 8           | run 1                   | 38                       | 1550                          |
|             | run 2                   | 29                       | 1725                          |
| 7           | run 1                   | 22                       | 1725                          |
|             | run 2                   | 24                       | 1250                          |
| 6           | run 1                   | 5                        | 2100                          |
|             | run 2                   | 4                        | 2050                          |
| 3           | run 1                   | seizure occurred at load | 1250                          |
|             | run 2                   | seizure occurred at load | 1200                          |
| 1           | run 1                   | 13                       | 1150                          |
|             | run 2                   | 14                       | 950                           |
| BIOHYDRAN   | run 1                   | 52                       | 1775                          |
|             | run 2                   | 59                       | not tested                    |
| ECOSAFE FR- | run 1                   | 8                        | 1600                          |
|             | run 2                   | 7                        | 1875                          |

The result from table IV suggest that the wear properties and extreme pressure properties of lubricants provided by

the invention compare favorably against commercially-available fluids. The results further indicate that the wear properties could be further improved by appropriate selection of anti-wear additives and extreme pressure additives.

Consideration must be given to the fact that although this invention has been described and disclosed in relation to certain preferred embodiments, obvious equivalent modifications and alterations thereof will become apparent to one of ordinary skill in this art upon reading and understanding this specification and the claims appended hereto. Accordingly, the presently disclosed invention is intended to cover all such modifications and alterations, and is limited only by the scope of the claims which follow.

15 I claim:

1. A liquid composition of matter that is useful as a hydraulic fluid or gear oil which consists essentially of:

a) a water-soluble polyoxyalkylene glycol monobutyl ether having a molecular weight of between 450 and 5000, said polyoxyalkylene glycol monobutyl ether being derived from n-butanol and a gaseous mixture of ethylene oxide and propylene oxide, and wherein the viscosity of the polyoxyalkylene glycol monobutyl ether is between 100 and 4000 in Saybolt Universal Seconds at 38° C.;

b) a carboxylic acid having between 6 and 18 carbon atoms per molecule of carboxylic acid; and

c) an amine.

20 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830

n-butanol, and a gaseous mixture of ethylene oxide and propylene oxide and is described by the general formula:



in which x is independently any whole integer between 0 and 5, including 0 and 5; y is independently any integer between 0 and 2, including 0 and 2; p is independently 0, 1, or 2; z is independently any whole integer between 0 and 5, including 0 and 5; and wherein m is an integer sufficient to provide a molecular weight between 450 and 5000, subject to the provisos that at least one of x and z is equal to at least one and that at least one of y and p is equal to at least one.

8. A composition according to claim 6 wherein the amounts of ethylene oxide and propylene oxide present in said water soluble polyoxyalkylene glycol are present in a ratio between of 0.25:1.00 to 4.00:1.00 on a molar basis, respectively, including every incremental hundredth therbetween.

9. A composition according to claim 7 wherein the amounts of ethylene oxide and propylene oxide present in said water soluble polyoxyalkylene glycol are present in a ratio between of 35:65 and 65:35 on a molar basis, respectively, and including every incremental hundredth therebetween.

10. A composition according to claim 8 wherein the amounts of ethylene oxide and propylene oxide present in said water soluble polyoxyalkylene glycol are present in a ratio of about 1:1 on a molar basis.

11. A composition according to claim 9 wherein the amounts of ethylene oxide and propylene oxide present in said water soluble polyoxyalkylene glycol are present in a ratio of about 1:1 on a molar basis.

12. A composition according to claim 6 wherein the amine is selected from the group consisting of: 2-(2-aminoethoxy) ethanol, monoethanol amine, diethanol amine, triethanol amine, 2-amino-2-methyl-1-propanol, 2-amino-2-ethyl-1,3-propanediol, mono-isopropanol amine, and di-isopropanol amine.

13. A composition according to claim 7 wherein the amine is selected from the group consisting of: 2-(2-aminoethoxy) ethanol, monoethanol amine, diethanol amine, triethanol amine, 2-amino-2-methyl-1-propanol, 2-amino-2-ethyl-1,3-propanediol, mono-isopropanol amine, and di-isopropanol amine.

14. A composition according to claim 12 wherein the amine is 2-(2-aminoethoxy) ethanol.

15. A composition according to claim 13 wherein the amine is 2-(2-aminoethoxy) ethanol.

16. A composition according to claim 1 wherein the carboxylic acid is selected from the group consisting of: octanoic acid, nonanoic acid, decanoic acid, dodecanoic acid, and mixtures thereof.

17. A composition according to claim 1 wherein said water-soluble polyoxyalkylene glycol is present in an amount of at least 92.0% of the total the composition on a weight basis.

18. A composition according to claim 1 wherein said carboxylic acid is present in any amount between 0.75 and 2.50% on a weight basis based upon the total weight of the liquid composition, including every hundredth percent therbetween.

19. A composition according to claim 1 wherein said extreme pressure additive is present in any amount between 0.50 and 2.00% of the total the composition on a weight basis, including every hundredth percent therebetween.

20. A composition according to claim 1 wherein said amine is present in any amount between 0.50 and 2.00% of the total the composition on a weight basis, including every hundredth percent therebetween.

\* \* \* \* \*